

April 11, 1933.

W. MENDEL

1,903,530

METHOD OF AND MEANS FOR MAKING ARTICLES FROM CELLULOID AND THE LIKE

Filed Nov. 14, 1928

FIG. I



FIG. II



FIG. III



INVENTOR:

WILLIAM MENDEL,

By *Arthur E. Taige*,  
Attorney.

## UNITED STATES PATENT OFFICE

WILLIAM MENDEL, OF BEVERLY, NEW JERSEY

## METHOD OF AND MEANS FOR MAKING ARTICLES FROM CELLULOID AND THE LIKE

Application filed November 14, 1928. Serial No. 319,280.

My invention relates to means for temporarily softening products of cellulose, such as celluloid, cellulose nitrate, cellulose acetate, and similar materials, to permit them to be shaped to form articles of manufacture; and particularly articles formed from primarily plane sheets.

It is the ordinary practice to soften such materials by immersion in water heated above the boiling point. However, the means for effecting such softening by that method are cumbersome to manipulate and result in deleterious distortion of the materials. Therefore, it is the present practice to soften celluloid by immersing it in an aqueous solution of acetone. However, altho the means for effecting such treatment are simpler and more easily operated; such treatment not only causes deleterious distortion of the celluloid, but renders the surface of the latter extremely sticky, so that the celluloid is difficult to manipulate and is marred by contact with any other substance while in such softened sticky condition.

Therefore, it is the object and effect of my invention to provide means for softening such materials without deleterious distortion thereof and without rendering them sticky.

I have discovered that acetone, which almost instantly dissolves celluloid immersed therein, may have such effect thereof limited and controlled by dilution of the acetone with any substance of the class known chemically as solvents, provided that such diluent has no deleterious effect upon the celluloid. For instance, such diluents may be any highly volatile hydrocarbon, but preferably carbon tetrachloride. Altho gasoline and naphtha may be used in lieu of carbon tetrachloride, the latter is preferable because it is not inflammable, like the hydrocarbons aforesaid.

For instance, in forming fountain pen tubes from primarily plane sheet celluloid, by the process disclosed in Letters Patent of the United States No. 1,661,451 granted March 6, 1928 to John N. Whitehouse for Improvement in method of and apparatus for making celluloid tubes; sheets of cel-

lloid 1, .010 of an inch thick and 4" x 12" in extent, such as indicated in Fig. I herein, are initially softened at their forward ends 2, to the extent indicated by the dotted line 3 in Fig. I, by successively laying each sheet, to that extent, upon a steam table, or other body, maintained at a temperature of about 225° F., until the celluloid is raised to approximately that temperature. The sheet is then stamped where thus softened to form a semi-cylindrical edge portion 5, as indicated in Fig. II, to fit the cylindrical mandrel 6 to which it may be cemented preliminary to rotating said mandrel and wrapping the sheet 1 in an evolute coil thereon, with its convolutions in contact. Such softening operation causes the sheet 1 to buckle at the region of the dotted line 3 because of the expansion of the portion 2 thereof by heat, and such distortion of the sheet 1 interferes with the formation of the tube 7 which is more or less corrugated at its inner surface 8, as indicated in Fig. III.

In accordance with my process, the sheet 1 may have its end portion 2 dipped into a solution of five per cent. acetone in ninety-five per cent. carbon tetrachloride up to the line 3, with the effect of softening the web 1 to such an extent that it may be readily wrapped upon the cylindrical mandrel 6, without distortion of the celluloid at the line 3 or elsewhere and, consequently, with considerable saving in the cost of production of tubes by said patented process.

In the formation of tubes by that process, from celluloid sheets .025 of an inch thick, I have found it convenient to employ a solution of ten per cent. acetone in ninety per cent. carbon tetrachloride, and the strength of the solution may be varied in accordance with the thickness of the material to be treated, to facilitate the softening operation. That is to say, altho celluloid of .025 inch thickness may be adequately softened in the solution aforesaid containing but five per cent. acetone; it is economical to use the stronger solution, because the latter effects the desired degree of softening in less time.

It is characteristic of the softening solutions aforesaid that altho the celluloid is

adequately softened thereby thruout its thickness, the surfaces of the celluloid which have been subjected to the action of such solution are not sticky, but feel dry to the touch.

Altho my invention is exemplified as aforesaid by the use of the softening solution upon plane sheets of celluloid, which are only partly dipped therein; of course, such sheets or other articles may be dipped in such a solution to any desired extent and for any desired length of time, according to the degree of softening thereof required; or any celluloid article may be otherwise subjected to the softening action of such a composition of acetone and hydrocarbon; for instance, by brushing or spraying such composition thereon. Moreover, the vapor from such a composition of acetone and carbon tetrachloride has a softening effect upon celluloid and similar substances; so that such softening effect may be attained without direct contact of the liquid composition with the article to be softened.

Either the softening liquid or fluid therefrom may be readily directed thru a flexible conduit to the area of the material to be softened.

Altho acetone is a preferable solvent for said celluloid and nitrate; I prefer to use ethyl acetate, or a mixture of alcohol and ether, for cellulose acetate. The latter is preferable to celluloid, in that it is noninflammable; and said solvents thereof may be diluted with carbon tetrachloride, or any other fluid which has no deleterious effect upon the material to be softened.

Therefore, I do not desire to limit myself to the precise details of construction, arrangement, or method of procedure herein set forth, as it is obvious that various modifications may be made therein without departing from the essential features of my invention, as defined in the appended claims.

45 I claim:

1. The method of softening celluloid, which consists in subjecting it to the action of a composition including acetone which has the capacity to penetrate and soften the celluloid, and an anhydrous diluent of the acetone which is miscible therewith but has no such effect upon the celluloid; containing such action until the celluloid is softened, and terminating such action before the celluloid is dissolved in said composition.

2. A method as in claim 1; wherein the diluent is a carbon compound.

3. A method as in claim 1; wherein the diluent is a highly volatile liquid carbon compound.

4. A method as in claim 1; wherein the diluent is a noninflammable carbon compound.

5. A method as in claim 1; wherein the diluent is carbon tetrachloride.

6. The method of softening without dissolving a product of cellulose, which consists in subjecting it to the action of a fluid including a solvent of said product having the capacity to penetrate and soften said product, and an anhydrous diluent of said solvent which has no such effect upon said product, continuing such action until the product of cellulose is softened, and terminating such action before the product of cellulose is dissolved in such composition.

7. The method of making a tube of celluloid from a primarily flat web, which includes dipping one end of said web into a solution of from five to ten per cent. acetone and ninety to ninety-five per cent. carbon tetrachloride until the dipped portion is softened to such an extent that it may be readily wrapped upon a cylindrical mandrel of the approximate diameter of the interior of the tube being formed; wrapping the softened end of the web upon such a mandrel and evolutedly winding the other portions of said web in convolutions on said mandrel which are in contact with each other.

In testimony whereof, I have hereunto signed my name at Burlington, New Jersey, this thirty-first day of October, 1928.

WILLIAM MENDEL.

95

100

105

110

115

120

125

130

CERTIFICATE OF CORRECTION.

Patent No. 1,903,530.

April 11, 1933.

WILLIAM MENDEL.

It is hereby certified that error appears in the printed specification of the above numbered patent requiring correction as follows: Page 2, line 52, claim 1, for "containing" read "continuing"; and that the said Letters Patent should be read with this correction therein that the same may conform to the record of the case in the Patent Office.

Signed and sealed this 16th day of May, A. D. 1933.

(Seal)

M. J. Moore,  
Acting Commissioner of Patents.